

July 10, 1973

J. E. MEE ET AL

3,745,046

METHOD FOR PRODUCING BUBBLE DOMAINS IN MAGNETIC  
FILM-SUBSTRATE STRUCTURES  
Filed Dec. 28, 1970



INVENTORS  
JACK E. MEE  
BY PAUL J. BESSER  
GEORGE R. PULLIAM  
DAVID M. HEINZ  
PERRY E. ELKINS  
*Joseph C. Koeninger*  
ATTORNEY

## 1

3,745,046

### METHOD FOR PRODUCING BUBBLE DOMAINS IN MAGNETIC FILM-SUBSTRATE STRUCTURES

Jack E. Mee, Paul J. Besser, George R. Pulliam, David M. Heinz, and Perry E. Elkins, Orange, Calif., assignors to North American Rockwell Corporation, El Segundo, Calif.

Filed Dec. 28, 1970, Ser. No. 101,785  
Int. Cl. H01f 10/06

U.S. Cl. 117—235

7 Claims

#### ABSTRACT OF THE DISCLOSURE

A method for producing a bubble domain in a magnetic single crystal garnet film-substrate structure is disclosed. The method involves the epitaxial deposition of an iron garnet film of the proper crystallographic orientation and having a positive magnetostriction constant on a garnet substrate in which the room temperature lattice constant of the film is larger than the room temperature lattice constant of the substrate, preferably by an amount less than 0.035 angstrom.

#### BACKGROUND OF THE INVENTION

##### (1) Field of the invention

This invention relates to bubble domains and more particularly to a method of forming a craze-free film having bubble domains therein.

##### (2) Description of prior art

Magnetic bubble domains in a sheet of magnetic medium, such as yttrium orthoferrite, are well known in the art and are described in U.S. Pat. No. 3,460,116 and others. Magnetic bubble domains in composite structures having a thin film of a single crystal iron garnet on an oxide substrate are disclosed in the co-pending patent applications to Mee et al., U.S. Ser. Nos. 16,446, filed Mar. 4, 1970 and now U.S. Pat. No. 3,645,788 and 16,447 filed Mar. 4, 1970. These co-pending patent applications are incorporated herewith.

Some of the bubble domain composite single crystal film-substrate structures reported in the prior art have had crazing, that is cracking, of the film, making them unsuitable for certain types of bubble domain device applications. Other iron garnet film-substrate structures were observed to have domains whose magnetization directions are in the plane of the film in contrast to the desired bubble domains whose magnetization directions are perpendicular to the plane of the film.

#### SUMMARY OF THE INVENTION

It is a primary object of this invention to provide an improved method of forming a single crystal iron garnet film-substrate structure having bubble domains therein.

It is another object of this invention to provide a method of forming a bubble domain film-substrate structure having a craze-free film surface.

These and other objects of this invention are accomplished by a method in which the uniaxial anisotropy necessary for bubble domain formation in a craze-free film-substrate structure is affected by proper control of the mechanical stress present in the film at room temperature. A specific step in the method involves depositing a single crystal iron garnet film of the proper crystallographic orientation and having a positive magnetostriction constant on a substrate in which the room temperature lattice constant of the film is larger than the room temperature lattice constant of the substrate preferably by an amount less than 0.035 angstrom.

## 2

An example of a preferred embodiment in accordance with this invention is to chemically vapor deposit a terbium iron garnet,  $Tb_3Fe_5O_{12}$ , film of the proper orientation and having a positive magnetostriction constant on a samarium gallium garnet,  $Sm_3Ga_5O_{12}$ , substrate. The lattice constant of the film is 12.441 angstroms which is 0.005 angstrom larger than the 12.436 angstrom lattice constant of the film.

Other objects and advantages of this invention will be apparent from the following detailed description wherein a preferred embodiment of the present invention is clearly shown.

#### BRIEF DESCRIPTION OF THE DRAWING

15 The drawing shows a magnetic bubble domain film-substrate structure made in accordance with the method of this invention.

#### DETAILED DESCRIPTION OF THE INVENTION

20 This invention involves a process in which a single crystal iron garnet material is chemically vapor deposited to form a film on a substrate. It is necessary that the single crystal material have the proper crystallographic orientation to take advantage of the positive magnetostriction. In addition the room lattice constant of the deposited film is larger than the room lattice constant of the substrate by an amount less than 0.035 angstrom. The resultant film-substrate structure has a craze-free film with bubble domains therein.

25 30 In general, the normal source of uniaxial anisotropy observed in magnetic materials is the crystal structure of the material. When single crystal platelets with positive magnetostriction constants ( $\lambda_{100}, \lambda_{112} > 0$ ), are under stress, the magnetostriction contribution tends to make the normal to the plane of the platelet an easy axis of magnetization if the platelet is in compression ( $\delta < 0$ ), and a hard axis if the platelet is in tension ( $\delta > 0$ ) where  $\lambda_{100}$  and  $\lambda_{111}$  are the saturation values of the linear magnetostriction constants along the  $\langle 100 \rangle$  and  $\langle 111 \rangle$  directions, respectively, and  $\sigma$  is the stress in the plane of the material.

35 40 The room temperature magnetostriction constants of selected iron garnets are listed in the following table.

| Iron garnet                 | Magnetostriction constant     |                               |
|-----------------------------|-------------------------------|-------------------------------|
|                             | $\lambda_{100} (\times 10^6)$ | $\lambda_{111} (\times 10^6)$ |
| $Sm_3Fe_5O_{12}$            | +21                           | -8.5                          |
| $Eu_3Fe_5O_{12}$            | +21                           | +1.8                          |
| $Gd_3Fe_5O_{12}$            | 0                             | -3.1                          |
| $Tb_3Fe_5O_{12}$            | -3.3                          | +12                           |
| $Dy_3Fe_5O_{12}$            | -12.5                         | -5.9                          |
| $Ho_3Fe_5O_{12}$            | -3.4                          | -4.0                          |
| $Er_3Fe_5O_{12}$            | +2.0                          | -4.9                          |
| $Tm_3Fe_5O_{12}$            | +1.4                          | -5.2                          |
| $Y_3Fe_5O_{12}$             | +1.4                          | -4.5                          |
| $Y_3Fe_5O_{12}$             | -1.4                          | -2.4                          |
| $Y_3Ga_{5.6}Fe_{4.4}O_{12}$ | -1.4                          | -2.4                          |
| $Lu_3Fe_5O_{12}$            | -1.4                          | -2.4                          |

55 Some of these iron garnet materials, for example,

60  $Tb_3Fe_5O_{12}$

and  $Yb_3Fe_5O_{12}$ , have both a negative and a positive magnetostriction constant. In the practice of this invention the crystallographic orientation of the garnet film must be chosen to take advantage of the positive magnetostriction constant. In the case with  $Tb_3Fe_5O_{12}$  material, the orientation would be  $\{111\}$ . With the  $Yb_3Fe_5O_{12}$  material, the orientation would be  $\{100\}$ .

65 70 The values of the magnetostriction constants of the iron garnet material, as well as its magnetization, can be varied by depositing a film containing a mixture of two or more pure iron garnets and/or by substituting other cations for iron ions.

It is understood that whether there is mixing and/or substitution or not, the condition for bubble domain formation in the iron garnet material,  $H_A/4\pi M_s > 1$ , has to be satisfied, where  $H_A$  is the uniaxial anisotropy field and  $4\pi M_s$  is the magnetization.

In magnetic oxide film-substrate structures formed by chemical vapor deposition, the dominant source of uniaxial anisotropy is the magnetostrictive effect resulting from the stress existing in the film. This stress is due to the difference between the lattice constants and the thermal expansion coefficients of the film and substrate and may be in the form of tension or compression.

This invention specifically covers a method of forming a bubble domain structure by depositing a magnetic single crystal garnet film of the proper orientation and having a positive magnetostriction constant on a substrate in which the film is in compression.

A co-pending application to Mee et al., Ser. No. 101,786, filed Dec. 28, 1970 covers a method of forming a bubble domain structure by depositing a magnetic single crystal garnet film of the proper orientation and having a negative magnetostriction constant on a substrate in which the film is in tension.

A co-pending application to Mee et al., Ser. No. 101,787, filing date Dec. 28, 1970 covers a second method of forming a bubble domain structure by depositing a magnetic single crystal garnet film of the proper orientation and having a negative magnetostriction constant on a substrate in which the film is in tension.

As shown in the drawing, an oxide substrate 10 is preferably subjected to a chemical vapor deposition step to provide a thin film of magnetic bubble domain material, film 12. The deposition step is carried out in accordance with the co-pending application, Ser. No. 833,268 filed June 16, 1969 and now abandoned, and assigned to the assignee of the present invention. This pending patent application is incorporated herewith by reference hereto. The film 12 may be deposited by sputtering techniques or by a liquid phase epitaxial process.

The substrate 10 is monocrystalline garnet having a  $J_3Q_5O_{12}$  formulation wherein the J constituent of the wafer formulation is at least one element selected from the group consisting of cerium, praseodymium, neodymium, promethium, samarium, europium, gadolinium, terbium, dysprosium, holmium, erbium, thulium, ytterbium, lutetium, lanthanum, yttrium, calcium, and bismuth; and the Q constituent of the wafer formulation is at least one element selected from the group consisting of indium, gallium, scandium, titanium, vanadium, chromium, manganese, rhodium, zirconium, hafnium, niobium, tantalum, aluminum, phosphorus, arsenic and antimony.

Examples of substrate materials are mixed yttrium gadolinium gallium garnet, gadolinium gallium garnet, aluminum substituted gadolinium gallium garnet, terbium gallium garnet, samarium gallium garnet, and dysprosium gallium garnet.

The film of the bubble domain material is a single crystal garnet film having a  $J_3Q_5O_{12}$  formulation wherein the J constituent of the film formulation has at least one element selected from the group of cerium, praseodymium, neodymium, promethium, samarium, europium, gadolinium, terbium, erbium, thulium, ytterbium, and lanthanum; the Q constituent of the film formulation is taken from the group consisting of iron, iron and aluminum,

iron and gallium, iron and indium, iron and scandium, iron and titanium, iron and vanadium, iron and chromium, and iron and manganese.

A preferred substrate material is samarium gallium garnet when the film material is terbium iron garnet.

In accordance with this invention, an iron garnet film of the proper orientation and having a positive magnetostriction constant is deposited on a garnet substrate in which the room temperature lattice constant of the film is larger than the room temperature lattice constant of the substrate, preferably by an amount less than 0.035 angstrom. The preferred difference between the lattice constants is of the order of 0.010 to 0.025 angstrom. When the lattice constant difference is about 0.035 angstrom or more, the compressive stress is so great that the compression relieves itself and the film is in tension due to the thermal expansion mismatch. When the film lattice constant is smaller than the substrate lattice constant, the film is in tension and there are no bubble domains since the normal to plane of the film is the hard magnetization axis and the domain magnetizations lie in the plane.

As previously discussed, the difference in the coefficients of thermal expansion between the film and the substrate contributes to the total stress present in the film. The thermal expansion stress contribution is within acceptable limits as long as the coefficient of thermal expansion of the substrate does not differ from that of the film by more than  $1 \times 10^{-6}/^{\circ}\text{C}$ . between  $25^{\circ}\text{C}$ . and  $1200^{\circ}\text{C}$ . A certain amount of mismatch between film-substrate room temperature lattice constants and/or thermal expansion characteristics is required in order to provide the stress which produces the uniaxial anisotropy necessary for bubble domain formation. If film and substrate are too closely matched in both lattice constant and thermal expansion, the proper stress necessary for bubble domain formation will not be achieved.

#### Example I

A [111] film of terbium iron garnet,  $\text{Tb}_3\text{Fe}_5\text{O}_{12}$ , having a lattice constant of 12.441 angstroms was deposited on a samarium gallium garnet,  $\text{Sm}_3\text{Ga}_5\text{O}_{12}$ , by chemical vapor deposition techniques. The lattice constant of the samarium gallium garnet was 12.436, which was smaller than that of the film by 0.005 angstrom. The resultant structure had a craze-free film which had bubble domains therein.

#### Examples II-IV

Examples I-IV are listed below in the following table. In Example II, a [111] terbium iron garnet film was deposited in accordance with this invention on a gadolinium gallium garnet in which the film lattice constant exceeded the substrate lattice constant at room temperature by 0.065 Å. The compressive stress due to the large lattice mismatch was relieved at the deposition temperature and the film is in tension due to the thermal expansion mismatch between film and substrate. This structure had no bubble domains in the film and also had crazing on the film surface. In Example III, the film is again in tension leading to domains whose magnetization lies in the film plane. Example IV shows a film in compression but having negative magnetostriction and again there were no bubble domains, only domains whose magnetization lies in the plane.

TABLE

| Example No. | Material <sup>a</sup>                                                | Lattice constant, <sup>a</sup> Å. | Material <sup>a</sup>                                    | Lattice constant, <sup>a</sup> Å. | Substrate lattice constant-film lattice constant, <sup>a</sup> Å. |               | Bubble domain | Domains in-plane | Crazing on film surface | Stress |
|-------------|----------------------------------------------------------------------|-----------------------------------|----------------------------------------------------------|-----------------------------------|-------------------------------------------------------------------|---------------|---------------|------------------|-------------------------|--------|
|             |                                                                      |                                   |                                                          |                                   | Substrate lattice constant, <sup>a</sup> Å.                       | Bubble domain |               |                  |                         |        |
| I.....      | $\text{Tb}_3\text{Fe}_5\text{O}_{12}$ <sup>b</sup>                   | 12.441                            | $\text{Sm}_3\text{Ga}_5\text{O}_{12}$                    | 12.436                            | -0.005                                                            | Yes.....      | No.....       | None.....        | Compression.            |        |
| II.....     | $\text{Tb}_3\text{Fe}_5\text{O}_{12}$ <sup>b</sup>                   | 12.441                            | $\text{Gd}_3\text{Ga}_5\text{O}_{12}$                    | 12.376                            | -0.065                                                            | No.....       | Yes.....      | Yes.....         | Tension.                |        |
| III.....    | $\text{Tb}_3\text{Fe}_5\text{O}_{12}$ <sup>b</sup>                   | 12.441                            | $\text{Nd}_{0.7}\text{Sm}_{2.3}\text{Ga}_5\text{O}_{12}$ | 12.452                            | +0.011                                                            | No.....       | Yes.....      | None.....        | Do.                     |        |
| IV.....     | $\text{Y}_3\text{Ga}_{1.2}\text{Fe}_{3.8}\text{O}_{12}$ <sup>c</sup> | 12.357                            | $\text{Tb}_3\text{Ga}_5\text{O}_{12}$                    | 12.347                            | -0.010                                                            | No.....       | Yes.....      | None.....        | Compression.            |        |

<sup>a</sup> [111] orientation.

<sup>b</sup> Positive magnetostriction constant.

<sup>c</sup> Negative magnetostriction constant.

We claim:

1. A method of producing a bubble domain containing film-substrate structure comprising the step of depositing a magnetic film of a single crystal material of the proper crystallographic orientation and having a positive magnetostriction constant on a substrate in which the magnetic film has a room temperature lattice constant which exceeds the room temperature lattice constant of the substrate at room temperature by an amount less than about 0.035 angstrom.

2. A method of producing a bubble domain containing single crystal iron garnet film-substrate structure comprising the step of depositing an iron garnet film of the proper orientation and having a positive magnetostriction constant on a substrate in which the iron garnet film has a room temperature lattice constant which exceeds the room temperature lattice constant of the substrate by an amount less than about 0.035 angstrom.

3. A method as described in claim 2 whereby the room temperature lattice constant of the substrate exceeds the room temperature lattice constant of the film by an amount between 0.010 and 0.025 angstrom.

4. A method as described in claim 3 whereby the room temperature lattice constant of the substrate exceeds the room temperature lattice constant of the film by an amount between 0.015 and 0.020 angstrom.

5. A method as described in claim 2 whereby said film is deposited by a chemical vapor deposition technique.

6. A method of producing a bubble domain containing film-substrate structure comprising the step of depositing

5 a terbium iron garnet film of the proper crystallographic orientation and having a positive magnetostriction constant on a substrate in which the film has a room temperature lattice constant which exceeds the room temperature lattice constant of said substrate by an amount less than about 0.035 angstrom.

7. A method as described in claim 6 wherein said substrate is a samarium gallium garnet.

10

#### References Cited

##### UNITED STATES PATENTS

|           |         |              |       |             |
|-----------|---------|--------------|-------|-------------|
| 3,617,381 | 11/1971 | Hanak        | ----- | 117—235     |
| 3,525,638 | 8/1970  | Archey       | ----- | 117—107.1 X |
| 3,486,937 | 12/1969 | Linares      | ----- | 117—235 X   |
| 3,429,740 | 2/1969  | Mee          | ----- | 117—235 X   |
| 3,131,082 | 4/1964  | Gambino      | ----- | 117—235     |
| 3,573,099 | 3/1971  | Moore et al. | ----- | 117—235 X   |
| 3,645,787 | 2/1972  | Mee et al.   | ----- | 117—240     |
| 3,645,788 | 2/1972  | Mee et al.   | ----- | 117—240     |

##### OTHER REFERENCES

Giess et al., IBM Tech. Dis. Bull. pp. 517, 117—235, vol. 13, No. 2, July 1970.

25 WILLIAM D. MARTIN, Primary Examiner

B. D. PIANALTO, Assistant Examiner

U.S. CL. X.R.

30 117—106 R; 340—174 TF, 174 M

UNITED STATES PATENT AND TRADEMARK OFFICE  
CERTIFICATE OF CORRECTION

PATENT NO. : 3,745,046  
DATED : July 10, 1973  
INVENTOR(S) : Jack E. Mee, et al.

It is certified that error appears in the above-identified patent and that said Letters Patent are hereby corrected as shown below:

Claim 3, line 2, change "substrate" to --film--;

line 3, change "film" to --substrate--.

Claim 4, line 2, change "substrate" to --film--;

line 3, change "film" to --substrate--.

Signed and Sealed this

Twenty-fifth Day of September 1979

[SEAL]

Attest:

LUTRELLE F. PARKER  
Attesting Officer      Acting Commissioner of Patents and Trademarks